

# UNITED STATES PATENT OFFICE.

WILLIAM H. ALLEN, OF DETROIT, MICHIGAN.

## RUST PREVENTING AND ARRESTING SOLUTION.

1,329,573.

Specification of Letters Patent. Patented Feb. 3, 1920.

No Drawing.

Application filed September 25, 1919. Serial No. 326,377.

To all whom it may concern:

Be it known that I, WILLIAM H. ALLEN, a citizen of the United States, and residing at Detroit, in the county of Wayne and State 5 of Michigan, have invented a new and Improved Rust Preventing and Arresting Solution, of which the following is a specification.

This invention relates to means for arresting and preventing the oxidation of the surfaces of articles of iron and steel, and its object is to provide a liquid compound which may be applied while cold to such surfaces by means of brushes or air currents, 15 or may be used as a dip or bath.

It has long been known that a weak aqueous solution of phosphoric acid and certain acid salts thereof will produce a surface of iron phosphates on articles of 20 iron and steel when left in the solution which is kept approximately boiling for a sufficient length of time, such surface being rust-proof under ordinary atmospheric conditions. But many structures of iron and 25 steel such as bridges and freight cars cannot be placed in a rust-proofing bath, and, after their surfaces are rusted, it is a very difficult matter to arrest oxidation. Brushing to remove the rust and then painting 30 has been found to work only moderately well, as the paint scales off and rusting often goes on under the paint.

Spraying with an active rust-proofing solution has been found to work better than 35 brushing and painting, especially if such spraying is followed by painting, but where the surfaces are covered with a heavy layer of rust, and especially where the surface is anywhere nearly upright so that the solution will adhere only as a very thin film, the action of the solution is not very satisfactory. This is particularly true for the reason that the liquid quickly dries and becomes ineffective.

40 I have found that deep rust can be completely altered, that is, changed to insoluble phosphates, by means of a solution of phosphoric acid or acid phosphates containing a small amount of inert miscible compounds 45 which are deliquescent or hydroscopic.

Such substances greatly retard the evaporation of the water from the rust-proofing solution and many will so thicken the solution that it will adhere to the metal in a layer of considerable depth as compared 55 with the very thin film usually obtained. Such inert substances have no apparent effect chemically, but serve to retain the water in such coating under atmospheric exposure, and such conditions bring about a 60 balancing of the reaction between the acid and the iron oxids and the metallic iron so that a totally different physical condition results. The phosphates of iron formed by said reaction are part of the surface of the 65 metal and constitute a rust-proof protecting surface.

I find that glycerin and certain carbohydrates such as glucose and levulose conform to the above conditions, and that good 70 results are obtained by using seventy parts of ordinary fifty per cent. strength phosphoric acid, twenty parts of glycerin or glucose and thirty parts of water, that is, the equivalent of thirty-five parts of pure 75 phosphoric acid, twenty parts of glucose or glycerin, and water sufficient to make one hundred parts, all by weight. This compound is applied and left for twenty-four hours, after which the article is washed 80 with strong soapy water and when dry, mineral lubricating oil may be applied or the surface may be painted. Where the surface is at an angle to the horizontal, the compound is liable to flow therefrom to a 85 greater or less extent so that in many cases a second and perhaps a third application may be necessary especially when the corrosion is deep seated.

These inert substances function as holders 90 of the water which acts as a catalytic to complete interaction between the acid and the base. The proportions set forth above may be varied within quite wide ranges, but those given seem to give the best results. 95

I claim:—

1. A compound for arresting and preventing the rusting of surfaces of iron and steel consisting of the equivalent of thirty-five parts of pure phosphoric acid, twenty parts 100

of glucose and water sufficient to make one hundred parts.

2. A compound for changing rust on surfaces of iron and steel to phosphates, consisting of phosphoric acid, water and a deliquescent carbo-hydrate.

3. A compound for changing rust on surfaces of iron and steel to phosphates, con-

sisting of acid phosphor compounds, water and an inert deliquescent substance.

4. A compound for changing rust on surfaces of iron and steel to phosphates, consisting of acid phosphor compounds, water and an inert hydroscopic substance.

WILLIAM H. ALLEN.